

J. M. LYNCH.  
METHOD OF MAKING DIES.  
APPLICATION FILED SEPT. 25, 1911.

1,160,179.

Patented Nov. 16, 1915.



WITNESSES.

Elizabeth C. Coyle  
Edith C. Hollbrook

INVENTOR.

John M. Lynch  
By his Attorney,  
Nelson & Conard.

# UNITED STATES PATENT OFFICE.

JOHN M. LYNCH, OF BEVERLY, MASSACHUSETTS, ASSIGNOR TO UNITED SHOE MACHINERY COMPANY, OF PATERSON, NEW JERSEY, A CORPORATION OF NEW JERSEY.

## METHOD OF MAKING DIES.

1,160,179.

Specification of Letters Patent. Patented Nov. 16, 1915.

Application filed September 25, 1911. Serial No. 651,254.

*To all whom it may concern:*

Be it known that I, JOHN M. LYNCH, a citizen of the United States, residing at Beverly, in the county of Essex and State 5 of Massachusetts, have invented certain Improvements in Methods of Making Dies, of which the following description, in connection with the accompanying drawings, is a specification, like reference characters on 10 the drawings indicating like parts in the several figures.

This invention relates to methods of making dies of the type used in connection with a clicking press for cutting upper leather 15 for boots and shoes.

More especially the invention relates to a novel method of making dies having lateral indentations or nicks in their cutting edges for the purpose of indicating the size 20 of the blanks cut out by the die, or for indicating amount of lap in assembling the blanks or the location of the lines of stitching.

It is an object of the present invention to 25 devise a method by which dies of this character may be produced by a process of casting as distinguished from the process there- 30 in described which involves forging and welding. The production of such dies on an economical basis presents many diffi- 35 culties, not only from the nature of the dies themselves and the accuracy required in their construction, but also because of the fact that rarely are two dies of exactly the same contour required. To meet these con- 40 ditions, therefore, it is important to devise a method whereby single dies of various shapes and sizes may be produced by following out a simple series of operations, 45 each requiring in itself little or no skilled labor and involving little waste of material.

It is an object of this invention to devise such a method.

The method comprises, in certain of its 45 important steps, the production of dies by first forming rough castings of cast iron having projecting ribs on one side thereof and subsequently converting the material 50 of the castings into a semi-steel which will possess substantially all the edge holding and shock resisting properties of mild steel, such properties as might be found in steel, 55 castings. By the present method, however, the expense incident to producing steel

castings is avoided and a finished die is produced which is not inferior to a cast steel die. Having produced a rough casting a cutting edge of the desired contour is formed by grinding or filing one edge of the 60 casting. A cutting edge of such shape as to form in the margin of each blank cut out by the die a notch of the required shape is then formed upon the end of the projecting rib. It is important that the notches in 65 the blanks should be disposed with great accuracy, particularly those which are intended for locating lines of stitching or lap of the blanks. The formation of a project- 70 ing rib on one side of the die casting facilitates the accurate location of the nick with respect to the previously formed cutting contour of the die by allowing the die maker sufficient material adjacent to the cutting edge to permit the location of the 75 nick to be varied slightly longitudinally of the edge of the die. On this account it is possible to compensate for inaccuracies be- 80 tween the pattern and the casting. Another advantage incident to this step of the 85 method is that material of superior quality is provided from which the nicks may be formed. It has been found that the cutting edges of the nicks, which are subjected to a serious wedging action in use, will main- 90 tain their shape a much longer time if cut out from a thick section of the casting, such as the ribs, than if formed from a thin casting which is likely to include surface scale.

Other advantages of the invention will be best understood and appreciated from the following description of a preferred manner of practising the method, the steps of which are illustrated in the accompany- 95 ing drawings, in which:

Figure 1 is a view in perspective of a block or slab from which the pattern is to be produced in position upon a table of a jig saw; Fig. 2 is a view in perspective of the partially sawed out pattern on the table of a band saw; Fig. 3 is a view in perspective of the completed pattern, a portion being broken away to show the shape of its cross section; Fig. 4 indicates the operation of wax finishing the pattern and shows the wax receptacle and polishing brush; Fig. 5 indicates the casting operation, and shows the mold and rough casting in cross section; Fig. 6 indicates the operation of de- 105 110

carburizing the castings, and shows several of them packed in iron scale in an annealing pot; Fig. 7 is a view in perspective of a complete vamp die.

5 In forming these dies a paper pattern is first provided having the outline of the blanks to be cut by the die, and therefore the desired outline of the cutting edge of the die. The paper pattern is furnished in duplicate 10 by the shoe manufacturer, each manufacturer having his individual styles. The outline of the paper pattern is indicated upon a board having a thickness equal to the height of the die. This operation may be 15 effected by the use of a grading machine which may be arranged to mark upon the board an outline determined by the paper pattern placed in the machine. If preferable, however, one of the paper patterns may 20 be pasted on the surface of the board. As but one or two dies are to be made from each pattern, a one-piece board will answer all the requirements, although from a laminated board composed of thin sheets glued 25 together a more durable pattern could be produced. In some cases however, it may be found practical to employ a slab of wax instead of a board as material from which to produce the pattern. Having indicated the 30 desired outline 14 upon the pattern block or slab 12, as shown in Fig. 1, the slab is perforated for the reception of the blade 16 of a scroll saw and placed upon the table 10. The interior line of the pattern, coinciding with the outline 14 is then sawed out. If it is desired to have the inner surface of 35 the die perpendicular to the cutting bed of the clicking press in sawing out the interior of the pattern the table 10 will be disposed 40 at right angles to the saw blade 16, so that the inner surface of the pattern will be perpendicular, but if an interior bevel is desired the table 10 may be set at a corresponding inclination to the saw. In case it is desired 45 to produce a die with size indicating indentations in its cutting edge projections 21 are left within the contour of the pattern, and in these projections 21 are subsequently carved corrugations 26 of the required shape 50 extending from one edge of the die to the other. If interior braces or brackets are required corresponding bridges 22 or ears 24 will be sawed out as an integral part of the pattern when the interior of the pattern 55 is being sawed. The partially sawed out pattern is then placed upon the table 18 of a band saw and the outer line of the pattern is cut out. The wedge shaped cross section desired in the die, indicated by the section 60 of the wooden pattern shown in Fig. 3, is conveniently secured in the pattern by disposing the table 18 at an angle to the saw blade 20. The pattern is sawed out with the edge uppermost which corresponds to the 65 cutting edge of the die, and in sawing the

outer line of the pattern it is necessary only to cause the saw to follow a line on the surface of the block or slab 12 about one thirty-second of an inch from the line 14 indicating the inner contour. On account of the 70 inclination of the table with respect to the saw the surface thus cut will diverge from the inner surface and will leave the back of the pattern substantially the width required in the corresponding portion of the die. 75 Having completed the sawing out operation the corrugations 26 are carved in the projecting portions 21 in any preferred manner. This may be done conveniently by special cutting tools shaped so that the corrugations 80 may be broached at a single operation. The thickness of the bridges 22 and brackets 24 is then reduced to the required dimensions by an end-cutting milling tool. Instead of sand-papering and smoothing the sawed out 85 pattern as has been usually done, the surface of the wooden pattern, sawed out in the manner hereinbefore described, is filled with wax and smoothed or wiped. As indicated in Fig. 4, the pattern is dipped in a receptacle 32 of melted wax, such as paraffin, for example, and its surface wiped and smoothed by the rotating brush 30. By the operation above outlined a pattern is produced having smooth surfaces which facilitate the 90 draft of the pattern from the sand of the mold and also in a large measure prevent the warping effect of dampness. Having produced the wooden pattern the casting 95 operation next takes place. As shown in 100 Fig. 5, the mold is formed entirely in the lower flask 44, while the plane surface of the cope 42 forms the back or pressure receiving surface of the die. The metal is gated into the sides of the die from the center, the casting being indicated by reference character 40. The material used for the casting will be a good grade of white iron. It is preferable that the analysis of the material should be as follows:—

|         |          |      |      |
|---------|----------|------|------|
| Total C | 2.75     | to   | 3.25 |
| Si      | 0.75     | to   | 1.25 |
| Mn      | 0.30     | to   | 0.50 |
| S       | not over | 0.10 |      |
| P       | not over | 0.23 |      |

110

115

When the rough castings have been produced and pickled as usual to remove the sand, they are packed with an oxidizing agent 52, such as iron scale, in a closed pot 50, as shown in Fig. 6, and subjected to heat sufficient to start a reaction between the oxidizing agent and the carbon of the castings, the heat being continued until most of the carbon has been extracted or converted to 120 temper carbon. It has been found that this result can be effected by subjecting the castings to a temperature from 1450° F. to 1600° F. for a period of about 48 hours. It should be borne in mind that by this opera- 125

tion the castings are not converted into malleable iron, but as distinguished from malleable iron, still retain some carbon in the form of hardening carbon by reason of which it is possible to harden and temper the castings as though they were formed of steel. Material having these characteristics is herein designated as semi-steel. When the decarburizing of the castings has proceeded to the proper point the pot 50 is allowed to cool slowly with its contents. The castings are thus annealed and are in such condition that they may be readily machined. The first step in this operation consists in bringing the narrow edge of the casting, which is to be the cutting edge of the die, into one plane. This is effected in any convenient manner, as, for example, by Gardner grinding upon the side of a rotating disk. The other surface of the die is then brought into a plane parallel to the plane of the cutting edge, and this operation may be performed conveniently upon several castings at once whereby a uniform height is secured in the dies. After the castings have been reduced to uniform height and opposite surfaces brought into parallel planes, they are ground or filed upon their inner and outer surfaces into their final shape, the contour of the cutting edge being frequently compared with the outline of the original paper pattern used in producing the wooden pattern for the casting operation. At this time the ribs or corrugations 60 on the inner surface of the castings are given their characteristic contour by filing on their inner surface and by filing notches 63 in the outer edge of the casting. The size indicating nicks may be shaped in accordance with any desired system such, for example, as the code disclosed in United States Letters Patent No. 990,248, granted April 25, 1911 on an application of T. H. Files. This method of producing the cutting indentations is of further importance, in that the corrugations which extend from one edge of the die to the other on the inside more than compensate for weakness in the die caused by filing the notches in its outer surface. The notches in the outer surface of the die need extend only a short distance back from the cutting edge. The bridges 62 and ears 64 require no machining except that the latter are drilled to receive the stab point markers 61. When the die has been given its final shape and sharpened to a cutting edge, it may be hardened and tempered in any preferred manner. A convenient manner of tempering the die is disclosed in my prior Patent No. 1,029,877, granted June 18, 1912, and consists in heating the die by floating it, edge down, in molten lead having a coating of charcoal, and then hardening the die in oil. A die constructed as above outlined may be left in a hard condition being drawn down only to a pale yellow temper. This is an important advantage of the invention in that it obviates the necessity of subjecting the hardened die to any considerable degree of heat, and therefore, lessens the liability of the finished die being distorted from its required shape.

Having now described my invention, I claim as new and desire to secure by Letters Patent of the United States:—

1. The method of making dies of closed contour having indicating notches therein, which consists in casting a rough die having projecting ribs on its inner side, converting the casting into semi-steel, finishing the casting, and interrupting the general contour of the die by forming cutting edges at the ends of the ribs and by cutting notches in the outer surface of the die opposite to the ribs which notches extend only a short distance from the cutting edge.

2. The method of making dies of closed contour having indicating notches therein, which consists in casting a closed frame having the general contour desired in the die and having projecting ribs on one side thereof, converting the casting into semi-steel by suitable heat treatment, after such heat treatment shaping a cutting edge at one edge of the casting, and interrupting the general contour of the cutting edge by forming transversely offset nicks in the ends of the projecting ribs.

In testimony whereof I have signed my name to this specification in the presence of two subscribing witnesses.

JOHN M. LYNCH.

Witnesses:

MABEL A. SWETT,  
CHESTER E. ROGERS.

Copies of this patent may be obtained for five cents each, by addressing the "Commissioner of Patents, Washington, D. C."